

# UNITED STATES PATENT OFFICE.

RICHARD PONNAY, OF LOS ANGELES, CALIFORNIA, ASSIGNOR OF ONE-FOURTH TO  
JOHN E. HUBBARD, OF LOS ANGELES, CALIFORNIA.

## BLASTING-POWDER.

1,033,927.

Specification of Letters Patent. Patented July 30, 1912.

No Drawing.

Application filed February 16, 1912. Serial No. 677,921.

To all whom it may concern:

Be it known that I, RICHARD PONNAY, a citizen of the United States, residing at Los Angeles, in the county of Los Angeles and State of California, have invented new and useful Improvements in Blasting-Powders, of which the following is a specification.

This invention relates to compositions of matter of the nature of blasting powders, for use in mine blasting and for allied purposes, and it has for its object to provide an improved blasting powder which will be superior in point of relative inexpensiveness and safety of production, safety in use, freedom from noxious fumes and products of combustion, and strength or explosive potential, and which will be generally superior in efficiency and serviceability and adaptability to varying conditions of use and service.

The above general objects and qualities of superiority I obtain by the selection and admixture of certain ingredients or materials, in certain more or less approximately predetermined relative proportions, the same being mixed together or combined as about to be stated.

The ingredients which I utilize, and the relative proportions of the same in a given quantity of the resultant composition or product, are as follows:—chlorate of potash, 45%; sugar (beet or cane), 30%; manganese oxid, 10%; charcoal, 7½%; and coal dust, 7½%; all of the above ingredients are separately ground or comminuted and moistened. The coal dust is first mixed with the chlorate of potash, and the other ingredients are then added and the whole mixture ground to produce a homogeneous mass. The product is then dried and re-ground and sized as desired, as to granulation, and is ready for use. If charcoal alone is employed, the combustion is too violent and is dangerous. By using coal dust with the charcoal the combustion is modified and kept within limits of safety.

The blasting powder constituted as above

recited is found to be of an explosive strength equal to that of commercial giant powder No. 2. It will not freeze, whereas giant powder freezes at approximately 50° Fahrenheit. It is safe to make, being free from liability to explode during the process of admixture of its ingredients. It is non-poisonous in itself, and also with respect to the products of combustion resulting upon its explosion, as it produces non-poisonous fumes, and even no fumes which are noxious or tend to choke or inconvenience miners and others using the powder in confined quarters. The powder is more inexpensive to produce than other blasting powders found at present on the market, and is easier to compound and manufacture. It will not ignite spontaneously or under friction, short of heavy impact with or between hard surfaces, and it will not explode unless confined. It requires no fulminate to cause its explosion, nor any detonation, the simple application of heat, by a spark or otherwise, being sufficient. If the powder becomes moistened it is not resultantly deteriorated, and when dried out, which may be safely done in an open vessel over heat, it has the same strength and explosive efficiency as before becoming moistened.

It will be noted that all of the ingredients utilized in compounding the blasting powder are relatively inexpensive, a number of them particularly so; and I am therefore enabled to produce a highly efficient blasting powder, having all of the qualities and attributes of superiority above outlined, which is lacking in the excessive cost attaching to the production and use of a great many explosives now found upon the market.

In conclusion, I do not desire to be understood as limiting myself to the specific provision, qualities, proportions, and method of admixture or compounding thereof as hereinabove set forth; but reserve the right to vary the same, in adapting the invention to varying conditions of service, or in complying with the exactions of various desiderata,

all without departing from the spirit of the invention and of the following claim:—

Having thus described my invention, I claim and desire to secure by Letters Patent:—

A blasting powder composed of chlorate of potash 45%, sugar 30%, manganese oxid 10%, charcoal 7½% and coal dust 7½%.

In testimony whereof, I have signed my name to this specification in the presence of two subscribing witnesses.

RICHARD PONNAY.

Witnesses:

C. P. WARDEN,  
RAYMOND IYES BLAKESLEE.